

## UNITED STATES PATENT OFFICE

2,222,562

## FINISHING COATED METAL SURFACES

Maurice D. German, Detroit, Mich., assignor to  
 Sno-Flake Products Company, Detroit, Mich.,  
 a corporation of Michigan

No Drawing. Application February 13, 1939,  
 Serial No. 256,221

2 Claims. (Cl. 51—281)

This invention relates broadly to the treatment of coated surfaces and is more particularly concerned with a method for smoothing the surfaces of coated metal objects. By the term, coat or 5 coating, as herein used, we mean films of paint, filler, sealer, enamel, lacquer, varnish and the like.

The abrading and leveling of coated surfaces of metal and other objects has long been a 10 problem, particularly where a finishing coat is later to be applied. The securing of a smooth finish on metal surfaces is difficult, due in part to the waves and other undesirable defects in such surfaces, caused by rolling or joining of two 15 pieces of metal together as by welding or soldering and the covering of other distinguishable surface flaws produced during the assembly of the object.

It has always been necessary to apply a type 20 of filler coat or surfacer to the metal and then sand this coat to as smooth a finish as possible before applying the final finish coat. In general, it is customary to apply a highly pigmented coating in preparing a smooth surface for the finish 25 coat. Such preliminary coatings have been ordinarily smoothed by hand or mechanically, employing an abrasive fixed on a fabric or paper backing. It is a well known fact that it is natural for the hand to follow the original contours of 30 the surface and the use of hand sanding does not always eliminate the depressed areas or natural waves, particularly when large areas are to be brought to a plane surface for the application of a finish coat. In addition to this, the use of an abrasive fixed to a permanent backing 35 frequently results in individual scratches of such depth that they are visible after the finish coat has been applied. A movable particle of abrasive will not cut as deeply as the same particle firmly affixed to a backing material and it has 40 been sought to take advantage of this fact by the use of water-in-oil emulsions of various types in which an abrasive was included, the emulsion being applied to the coated surface to be 45 smoothed and a mechanical means being employed in an endeavor to level down the surface. However, the use of such oily emulsions has not become general, because they are not entirely satisfactory in operation and, primarily, because 50 the residue from the abrading operation is difficultly removable from the surface, involving appreciable expense, and usually requiring a solvent wash with its attendant health hazard and solvent recovery problems.

55 I have now found that the foregoing disad-

vantages are obviated and coated metal surfaces satisfactorily abraded and leveled by applying a petroleum distillate-free, water-dispersive composition, containing a relatively finely divided abrasive, to the coated surface; then mechanically abrading down and leveling the surface as with a polishing wheel; and thereafter water-washing, as by a spray or sponging, the so-treated surface to remove substantially therefrom the residual product of the abrading step 10 before it has appreciably dried. This residual product will comprise the unused portion of the abrasive composition applied, that portion of the coating which has been cut away by the action 15 of the abrasive, and may include reaction products of the abrasive composition with the coating.

This improved process results in a uniformly smooth surface, free from pits, scratches, and other blemishes and devoid of oily films and 20 residues of a nature prejudicial to the application of additional layers or coats of finishing enamel, lacquer and the like.

An essential step, according to my invention, 25 is the water-washing of the treated surface to remove the residual product of the abrading step before it has appreciably dried. In order to accomplish satisfactorily this step, it is necessary that the actual abrading step be carried out at such a rate that the residue retains a substantial 30 amount of water while in contact with the surface under treatment. Once dried, this residue is difficult to remove. My process is essentially a wet-grinding process and it is desirable that the surface to be abraded and leveled be 35 thoroughly water-wet before the abrasive composition is applied thereto. However, where it is expedient to have a dry coated surface, the composition may be diluted with sufficient water so that the actual abrading step will be carried 40 out in the presence of sufficient moisture to be termed a wet-grind.

As a suitable abrading composition, we may 45 employ a material consisting essentially of a relatively finely divided abrasive, a water-soluble detergent, and water. Preferably a bodying agent is used. The quantities of the aforesaid materials are in such proportions that the composition is relatively viscous or weakly adhesive and is adapted to be readily applied to and retained on the coated surface to be leveled or on the working surface of a mechanical polishing means. In certain instances, it is desirable to employ an anti-foaming agent in the composition 50 and in other instances, a hygroscopic substance 55

- or a wetting agent may be incorporated in the composition. The proportions of the ingredients are not extremely critical but the abrasive should be in the order of between 80 and 325 screen 5 mesh particle size. The detergent must be completely water-dispersive and of sufficient body to serve both as a lubricant and binding agent in the composition. This latter statement with respect to the detergent is particularly true where 10 a bodying agent such as bentonite is not employed in the preparation of the composition.
- A representative composition particularly suitable for use in leveling filler coat on automobile bodies contain between about 55 and 80 15 parts by weight of an emery powder of about 120-220 mesh; between about 3 and about 5 parts of an alkali metal higher fatty acid soap, such as sodium oleate-stearate and between about 0.2 and about 0.5 parts of bentonite; together with sufficient water to produce a relatively viscous paste, e. g., from 15-30 parts. The compounding of the foregoing composition is ordinarily carried out by thoroughly intermixing the abrasive substance, bodying agent, and soap, 20 in the presence of a portion of the water, e. g., 50 per cent, which will be present in the final composition. After the ingredients are thoroughly co-mingled, the balance of the water is incorporated with the concentrate.
- After this composition has been applied to the 25 coated surface to be leveled, the surface is abraded, for example, with a rotary disk of which the contact surface is a fairly rough textile material, stretched over a spongy base, such as 30 rubber, sponge rubber, or felt pad. The preferred speed of the wheel is dependent in part on the hardness of the coating to be leveled, for example, speeds of about 900 R. P. M. may be employed on relatively highly pigmented coats 35 while speeds ranging up to 1760 R. P. M. may be used on low pigmented coats.

Among the abrasive materials which may be used in the preparation of my composition are: emery, silicon carbide, aluminum oxide, and the like. The sodium and potassium soaps of fatty acids such as elec, stearic, lauric, and the like, are useful as detergent substances, although I prefer to use the sodium salts because of their better bodying action. Other common detergent 45 materials such as the alkali metal salts of sulphonated hydrocarbons and sulphonated higher aliphatic alcohols may be substituted wholly or in part for the fatty acid soaps.

In certain instances it is desirable that bodying agents be included in the composition. While I prefer to employ bentonite, such materials as gum tragacanth or starch may be substituted therefor. Where lacquer base or other difficultly 50 wettable coatings are to be leveled, it is advan-

tageous that a wetting agent such as sulphite pulp waste liquor, alcohol, or similar product be incorporated, generally in amount ranging up to 1 to 2 per cent by weight of the composition. Along with such wetting agent a hygroscopic or 5 evaporation retarding material such as glycerol, ethylene glycol, diethylene glycol, and the like, may be incorporated in amount up to 3 per cent by weight. This results in such a reduction of the evaporation rate of moisture from the composition as prevents the "setting up" or hardening of residual abrasive prior to the water-washing step. Anti-foaming agents such as pine oil 10 and the like may be employed if desired.

My process provides a rapid and economical 15 way of abrading and leveling down coated surfaces and eliminates the disadvantages inherent in the hand or mechanical abrading of such surfaces with a fixed abrasive.

Compositions prepared within the foregoing 20 proportions have been employed in processing coatings on automobile bodies in commercial production in accordance with the method herein set forth.

Other modes of applying the principle of my 25 invention may be employed instead of those explained, change being made as regards the method herein disclosed, provided the means stated by any of the following claims or the 30 equivalents of such stated means be employed.

I therefore particularly point out and distinctly claim as my invention:

1. The method of smoothing and leveling the 35 surface of a highly pigmented pre-coating on an automobile body which comprises applying a petroleum distillate-free composition containing relatively finely divided abrasive, a water-soluble agent having a weak adhesive and a detergent effect, and water to said coated surface, mechanically abrading down and leveling the coating 40 on said metal surface utilizing a power-driven tool, and thereafter water-washing the coated surface to remove the residual product of the abrading step before it has appreciably dried.

2. The method of smoothing and leveling the 45 surface of a highly pigmented pre-coating on an automobile body which comprises applying a petroleum distillate-free composition containing relatively finely divided abrasive, a water-soluble agent having a weak adhesive and a detergent 50 effect, and water to said coated surface, mechanically abrading down and leveling the coating on said metal surface utilizing a power-driven wheel of which the contact surface is a fairly rough textile material backed by a resilient base, 55 and thereafter water-washing the coated surface to remove the residual product of the abrading step before it has appreciably dried.

MAURICE D. GERMAN.